

**METHOD OF REMOVING OXYGEN FROM  
TITANIUM METAL**

Eugene Wainer, Cleveland Heights, Ohio, assignor to  
Horizons Titanium Corporation, Princeton, N. J., a  
corporation of New Jersey

No Drawing. Application November 8, 1955  
Serial No. 545,790

6 Claims. (Cl. 148—13.1)

This invention relates to a process for removing oxygen as a contaminant from titanium containing material such as metallic titanium scrap or titanium alloy scrap. More particularly, it relates to a process in which oxygen containing metallic titanium or titanium alloys is reacted with one or more alkali metal fluotitanates in which the titanium is tetravalent, the reaction being carried out in the presence of carbon. The products of the reaction include a titanium metal product in which the oxygen content is substantially lower than that originally present therein, one or more complex alkali metal titanium fluorides in which the titanium has a valence of at least two and less than four and one or more gaseous materials from the group consisting of carbon monoxide, carbon dioxide and oxygen.

Various expedients have been suggested in the past for the removal of oxygen from titanium. Because of the tenacity with which oxygen is held in combination, most of these suggestions have involved melting the oxygen contaminated titanium and reaction of the oxygen with a powerful reducing agent such as an alkali metal or alkaline earth metal or with carbon under a high vacuum. Such suggestions require expensive reagents and complicated apparatus resistant to attack by molten titanium.

In a copending application, Serial No. 455,068, filed September 9, 1954, by Merle E. Sibert and Quentin H. McKenna, now United States Patent Number 2,723,182, there are disclosed similar reactions involving the various oxides of titanium, carbon and the alkali metal fluotitanates in which the titanium is tetravalent.

I have now discovered that the techniques therein disclosed are applicable to the purification of titanium metal or titanium alloys, whereby the removal of substantial amounts of oxygen may be effected at temperatures well below the melting point of the metal or alloy and whereby lower valent titanium halides may also be obtained as a valuable product of the reaction.

In accordance with my invention the oxygen content of contaminated metallic titanium or titanium alloys may be substantially diminished and even entirely removed by means of a simple thermal reaction between the contaminated metal, carbon and an alkali metal fluotitanate, in which the titanium has a valence of four. In my process the impure metallic material is immersed in a fused salt melt consisting of one or more alkali metal fluotitanates preferably maintained under an atmosphere which is inert with respect to the reactants. The reaction is carried out in the presence of carbon, provided in any convenient form, e. g. as pellets or as powder distributed throughout the melt, or as the vessel containing the fused melt. I prefer to operate at a temperature between 780° C. and about 1150° C. It is desirable to include one or more alkali metal chlorides, i. e. sodium, potassium or lithium chloride, in the reaction mixture as a diluent salt. As a result of the reaction one or more alkali metal-titanium double fluorides in which the titanium has a valence of less than four is produced and the oxygen content of the

metallic titanium is diminished. The metallic titanium is removed from the reaction mixture as a solid and is readily separated from the other solid materials such as carbon in the system. The alkali metal-titanium double fluoride product of the reaction may be recovered from the reaction residue either before or after the purified solid metallic material and any other solids present have been removed. The lower valent product is separated either by aqueous separation techniques or in the form of a molten bath of the product salt.

The alkali metal fluotitanates useful in the practice of the invention include sodium fluotitanate, potassium fluotitanate and lithium fluotitanate. In order to avoid undesirable side reactions and possible contamination of the product, the fluotitanate employed should be of recrystallized quality. That is to say, the fluotitanate should be substantially free of silica and metallic impurities and should contain less than about .01% water and .01% insolubles. Because of the relative cheapness and availability of potassium fluotitanate, I presently prefer to use this fluotitanate in the process. Therefore, in the interest of simplicity, the invention will be described in connection with the use of potassium fluotitanate as a representative of all metal alkali fluotitanates. However, it should be kept in mind that what is said with respect to potassium fluotitanate applies equally to the other alkali metal fluotitanates. Moreover, although the use of diluent alkali metal chlorides may not be specifically set forth, all reaction mixtures hereinafter referred to may contain as diluents alkali metal chlorides up to an amount equal molecularly to about the amount of alkali fluotitanate employed. Substantially chemically pure sodium, potassium and lithium chlorides suitable for use as diluents are available commercially. The alkali metal fluorides are not desirable diluents in the reaction mixture because of their ability to dissolve titanium oxides with the resulting formation of titanium oxy-fluorides. Bromides and iodides of the alkali metals do not dissolve titanium oxides but these halides form unstable titanium bromides and iodides which decompose or disproportionate at high temperatures to evolve tetra-bromides and tetra-iodides of titanium.

The metallic titanium to be purified is in any form having a large surface area to weight ratio. Preferably, it is in the form of powder, turnings, clippings, shavings or small pieces of light gage plate rather than in the form of bulky pieces of considerable thickness. As is conventional in the processing of such scrap, any extraneous coatings should be removed from the scrap and organic residues should also be removed, for example by degreasing with trichloroethylene. The processed scrap, freed from dirt and other gross impurities is next reduced to small pieces by chopping, shredding, or other suitable procedure preparatory to charging same into the reaction mixture.

The carbon employed should also be very pure and is preferably very finely divided in order that it may be readily dispersed throughout the reaction mixture. A suitable source of carbon is lampblack which has been calcined at a temperature of at least 1500° C. in a high vacuum prior to adding it to the reaction mixture.

The proportions of the several ingredients are not critical, but I have found it desirable for the amount of carbon present to exceed the amount of oxygen contained in the mixture. Because of the difficulty inherent in bringing the carbon and the oxygen contaminated metallic portion of the charge into intimate contact, I prefer to provide at least about 2½ atoms of carbon for each atom of oxygen in the mixture. Under the conditions of the process, the several ingredients interact to produce complex potassium and titanium fluorides in which the titanium has a valence less than four and to remove oxygen from the metal.

The reaction between the oxygen contaminated metal, carbon and potassium fluotitanate is carried out by bringing the metal and carbon into contact with potassium fluotitanate in an atmosphere inert with respect to the reactants at a temperature above the melting point of the fluotitanate but below that at which the resulting lower valent complex titanium salts decompose or disproportionate. The reaction will proceed to some extent just above the melting point 772° C. of pure potassium fluotitanate and is accelerated with increasing temperature. However, at temperatures of about 1200° C. or higher excessive decomposition and disproportionation are encountered. Accordingly, a temperature within the range of about 780° to 1150° C. and preferably within the range of about 780° to 1100° C. is useful in the practice of the invention. Within this range temperatures between about 780° to 900° C. result in the formation of trivalent alkali metal titanium fluorides, while temperatures in excess of about 900° C. favor the formation of divalent titanium fluorides.

It is essential that the reaction be carried out in an atmosphere which is inert to the reactants. The presence of even a trace amount of oxygen or moisture in the atmosphere will result in contamination and serious loss in yield of the desired product due to the formation of oxy-fluorides. Moreover, the reaction is accompanied by the evolution of carbon monoxide from the reaction mixture. Therefore, it has been found advisable to conduct the reaction in an actively pumping vacuum, or in an atmosphere composed of a dry monatomic gas, such as argon, which is continuously cycled through the reaction chamber to withdraw evolved carbon monoxide therefrom.

With the establishment of such an inert atmosphere, the reaction between the oxygen interstitially contained by the titanium metal or titanium base alloy material may be represented by an equation along the following lines:



Any suitable inert atmosphere furnace may be used for carrying out the process of my invention. One such furnace construction comprises a steel pot having an open top which can be sealed with a gas-tight lid. Advantageously, the steel pot is internally insulated with a refractory silicious powder held in place against the walls of the pot by means of a graphite liner. An internal heating element is provided, advantageously comprising a graphite resistance element adapted to surround the graphite reaction vessel. The graphite reaction vessel containing the reactants is disposed within the graphite resistance element which, in turn, is centrally positioned in the insulated pot. The necessary electrical connections to the heating element, and the necessary valves and inlet and outlet pipes for the establishment of the inert atmosphere within the furnace, are provided in the gas-tight lid of the steel pot.

To establish an inert atmosphere in the furnace, I presently prefer first to evacuate all of the air from within the furnace, and then to introduce dry argon gas into the furnace, repeating the cycle of evacuation of the atmosphere and replacement with argon gas at least two times. After flushing out the interior of the furnace in this manner, a flow of dry pure argon gas into and out of the furnace is established in order to sweep from the atmosphere in the furnace any carbon monoxide evolved from the reactants in the course of the reaction.

The reactants are heated in an inert atmosphere. A furnace such as that described is used to bring the re-

actants up to a reaction temperature within the range of about 780° to 1150° C. The reactants are held at this reaction temperature for a period of time sufficient to insure that the reaction has gone as close to theoretical completion as the reaction conditions permit. The time required for substantial completion of the reaction depends upon the extent of contamination of the metal, the intimacy of contact between the carbon and the small pieces of contaminated metal, and the temperature of the reactants. A reaction time of from five to ten hours is usually sufficient for the usual amount of oxygen found in commercially available impure titanium sponge or scrap.

On completion of the reaction the fused salt mass is filtered through a porous graphite or carbon filter, thus separating the molten salt from any residual solid materials such as carbon, carbides, titanium metal and oxy-fluorides. The purified titanium metal is easily separated from the remaining solids by washing with water or dilute acids. The molten salt filtrate may then be used directly or in admixture with additional diluent alkali metal chlorides in electrolytic processes for the production of titanium metal. The fused salt bath filtration procedure is particularly valuable in the preparation of divalent titanium fluorides, or mixtures of divalent and trivalent titanium fluorides. Divalent titanium fluoride is not generally amenable to aqueous treatment due to the strong reducing properties of divalent titanium salts. Heavy losses in yield can be expected even in highly buffered solutions. Accordingly it is preferable to recover the titanium difluoride containing product in the form of a fused salt bath in which the divalent titanium is present either in simple or complex difluoride compounds.

In an alternative procedure the molten salt filtrate is allowed to cool. The solidified salt cake thus recovered is reddish brown to greyish lavender in color and may contain, besides the lower valent titanium fluorides produced by the reaction, unreduced normal potassium fluotitanate, diluent alkali metal chlorides and any other fusible products that may have formed in the course of the reaction. The lower valent titanium fluoride product can be recovered from the reaction residue by wet chemical treatment.

The recovery of the lower valent titanium product by aqueous procedures is limited in practice to trivalent titanium fluorides. The product salt cake is first crushed to a fine powder and then is leached with cold dilute hydrochloric acid to dissolve the complex potassium salts of lower valent titanium fluorides which are soluble therein, leaving undissolved any potassium fluotitanate or other insolubles. A clear green liquor (characteristic of trivalent titanium solutions) is obtained as the result of the leaching operation, and this liquor is thereupon filtered to remove any insoluble matter. A saturated solution of sodium fluoride is added to the green filtrate while stirring the filtrate until the color changes permanently from green to brownish violet. The solution is then warmed gently (i. e. to a temperature of about 40° to 50° C.), whereupon tannish lavender crystals precipitate out of the solution leaving a violet colored supernatant liquid. The precipitated crystals are recovered by filtering the liquid, and the violet filtrate is again treated with a saturated solution of sodium fluoride. Upon addition of the sodium fluoride solution with stirring, the violet solution gradually becomes substantially colorless, at which point a slight turbidity develops. Gentle warming causes tannish violet colored crystals to precipitate from the solution leaving a water white supernatant liquid. The second batch of precipitated crystals are recovered by filtration and both batches are then washed with distilled water and dried at 105° C.

Although the exact structures of the complex lower valent titanium fluorides are not known with certainty, it has been found that the sodium fluoride derivatives

obtained as the first and second precipitates from the green liquor have completely different X-ray patterns, apparently indicative of different sodium fluoride and potassium fluoride contents. However, irrespective of their precise structure, the lower valent titanium fluoride products obtained by the practice of my invention is free from titanium dioxide, titanium carbide, potassium fluotitanate, and normal sodium and potassium fluorides and chlorides. These reduced titanium products are therefore available for subsequent use in a highly pure state. The titanium difluoride and trifluoride products of the process are useful for a variety of purposes including commercially important processes for the preparation of titanium metal.

The following examples are illustrative but not limitative of the practice of my invention:

*Example I*

A graphite crucible was charged with a mixture consisting of 500 grams of titanium clippings having an oxygen content of 0.28%, 700 grams of dry recrystallized potassium fluotitanate and 25 grams of -325 mesh (Tyler Standard) lampblack. The crucible was heated to a temperature of about 850° C. in an inert atmosphere furnace in which a continuously changing argon atmosphere had been established. The reaction mixture was stirred from time to time to insure that the lampblack contacted the metal and the fluotitanate throughout the mixture. The crucible was maintained at the reaction temperature for 4 hours. The mixture was then filtered through a perforated graphite plate pierced with a number of fine orifices, while still in an argon atmosphere. The separated solids and the molten salt filtrate were allowed to cool in the furnace. When the temperature had fallen to below 200° C., the argon supply was disconnected and the furnace was opened. The separated solids were washed with water and then with alcohol. The purified metal separated cleanly from the carbon lampblack and other non-molten bath constituents. The metal product analyzed 0.08% oxygen. Two buttons were prepared by arc melting a sample of the original scrap and of the purified scrap. The Brinell hardness of the two samples were 240 and 150 respectively.

The filtrate was observed to have a reddish color. It was ground to a fine powder. A representative sample of the ground powder was analyzed of titanium and was found to contain 25.0% titanium by weight. Since pure  $K_2TiF_6$  contains 19.9% by weight of titanium, the titanium content of the salt product represented an increase of 5.1% of the titanium content, over the original content. The titanium content of a compound such as that produced by the reaction of the first of the two previous equations is 25.0%. Thus for 100% completion of the reaction shown, the titanium content of the salt would increase by 5.1%. From the result obtained, it would appear that the reaction proceeded about 100% towards completion.

A portion of the ground powder was digested in a cold solution of HCl (3%) for about one hour. The soluble portion produced a clear green solution, which was filtered to remove insolubles therefrom. A saturated solution of sodium fluoride was then added slowly to the clear green filtrate, while stirring the filtrate, until the color changed permanently from green to brownish violet. The violet liquor was then warmed to 40° C., whereupon a lavender precipitate settled out. Heating was continued until the temperature of the solution reached 90° C. to keep dissolved and unreacted potassium fluotitanate in solution. The hot aqueous slurry was then filtered to recover the insoluble lavender crystals. To the clear lavender filtrate an additional amount of the saturated solution of sodium fluoride was added until the liquor became nearly colorless and a slight turbidity developed. The solution was again warmed to 40° C., whereupon a lavender precipitate

again settled out leaving a water white supernatant liquid. Both batches of fine violet crystals were then washed with distilled water and dried at 105° C. for 2 hours. The reducing properties of the dry lavender crystals indicated that lower valent titanium was present.

It should be pointed out that both the insoluble residue from the initial cold hydrochloric acid leaching step and the final filtrate from the titanium fluoride precipitation step contained some unreacted potassium fluotitanate. This material can be recovered from the insoluble residue by hot water leaching, and from the leach liquor and the final filtrate by evaporation and concentration operations. Thus, unreacted potassium fluotitanate is recoverable and can be dried and recycled through the process. After recovery of the unreacted potassium fluotitanate from the insoluble residue, the remaining titanium content thereof, made up of titanium oxides and oxyfluorides, is best recovered by digesting the residue in sulphuric acid. The resulting sulfate solution is diluted, filtered to remove free carbon and other insolubles, and is neutralized to precipitate titanium dioxide.

*Example II*

25 A graphite crucible was charged with a mixture of 500 grams titanium plate scrap having an average oxygen content of 0.28%, 700 grams of dry recrystallized potassium fluotitanate and 25 grams of -325 mesh (Tyler Standard) lampblack. The crucible was heated to a temperature of about 950° C. in an inert atmosphere furnace in which a continuously changing argon atmosphere had been established. The reaction mixture was stirred from time to time to insure that the lampblack contacted the metal and the fluotitanate throughout the mixture. The crucible was maintained at the reaction temperature for 12 hours. The mixture was then filtered through a perforated graphite plate pierced with a number of fine orifices, while still in an argon atmosphere. The separated solids and the molten salt filtrate were allowed to cool in the furnace. When the temperature had fallen to below 200° C., the argon supply was disconnected and the furnace was opened. The separated solids were washed with water and then with alcohol. The purified metal separated cleanly from the carbon lampblack and other non molten bath constituents. The metal product analyzed 0.06 oxygen. Two buttons were prepared by arc melting a sample of the original scrap and of the purified scrap. The Brinnell hardness of the two samples was 240 and 140 respectively.

50 The filtrate was ground to a fine powder after it had solidified and was analyzed for titanium. The salt product was found to contain 27.0% of titanium by weight, which represents an increase of 7.1% over the original titanium content.

55 The remainder of the ground salt cake was then mixed with sodium chloride in the ratio of about 5 parts by weight of sodium chloride to 1 part by weight of the salt cake. The resulting mixture was introduced into a suitable vessel and melted therein. When the mixture was molten electrodes were inserted into the melt and an electrolyzing current was initiated between the electrodes. The electrolysis was performed under an inert atmosphere and titanium metal was produced at the cell cathode.

60 It is apparent from the foregoing description and the examples accompanying same that there has been disclosed a novel and useful process for removing oxygen from oxygen-containing metallic titanium material other than the oxides of titanium, whereby the titanium metal is upgraded to the point that it may be readily fabricated by conventional metal working techniques after it has been reconstituted into the form of an ingot or slab product. In addition, as a by-product of the reaction, there is also contained a lower valent complex alkali metal titanium double fluoride, which is useful for a variety of

purposes including the electrolytic recovery therefrom of metallic titanium.

I claim:

1. The method of removing oxygen from oxygen containing titanium metal which comprises bringing together in the presence of carbon a molten alkali metal-titanium double fluoride, in which the titanium is tetravalent and a solid impure titanium metal interstitially containing oxygen at an elevated temperature within the range of about 780° C. to about 1150° C. under an inert atmosphere, and recovering from the reaction mixture the solid titanium metal with a diminished oxygen content and separately recovering at least one resulting alkali metal-titanium double fluoride in which the titanium has a valence less than four.

2. The method of removing oxygen from oxygen containing titanium metal which comprises bringing together in the presence of carbon a molten alkali metal-titanium double fluoride, in which the titanium is tetravalent and a solid impure titanium metal interstitially containing oxygen at an elevated temperature within the range of about 780° C. to about 1150° C. under an inert atmosphere, and separating the solid titanium metal with a diminished oxygen content from the reaction mixture.

3. The method of removing oxygen from oxygen containing titanium metal which comprises bringing together a molten alkali metal-titanium double fluoride, in which the titanium is tetravalent and a solid impure titanium metal interstitially containing oxygen in the presence of about 2½ mols of carbon for each mol of oxygen in the titanium at an elevated temperature within the range of about 780° C. to about 1150° C. under an inert atmosphere, and recovering from the reaction mixture the solid titanium metal with a diminished oxygen content.

4. The method of removing oxygen from oxygen containing titanium metal which comprises bringing together in the presence of carbon a molten alkali metal-titanium double fluoride, in which the titanium is tetravalent and a solid impure titanium metal interstitially containing oxygen at an elevated temperature within the range of about 780° C. to about 900° C. under an inert atmos-

phere, and recovering from the reaction mixture the solid titanium metal with a diminished oxygen content and separately recovering at least one resulting alkali metal-titanium double fluoride in which the titanium has a valence of three.

5. The method of removing oxygen from oxygen containing titanium metal which comprises bringing together a molten alkali metal-titanium double fluoride, in which the titanium is tetravalent and a solid impure titanium metal interstitially containing oxygen in the presence of carbon at an elevated temperature within the range of about 900° C. to about 1150° C. under an inert atmosphere, and recovering from the reaction mixture the solid titanium metal with a diminished oxygen content and separately recovering at least one resulting alkali metal-titanium double fluoride in which the titanium has a valence of two.

6. The method of removing oxygen from oxygen containing titanium metal which comprises bringing together in the presence of carbon a molten alkali metal-titanium double fluoride, in which the titanium is tetravalent and a solid impure titanium metal interstitially containing oxygen, there being present at least about 2½ mols of carbon for each mol of oxygen in the titanium metal at an elevated temperature within the range of about 780° C. to about 1150° C. under an inert atmosphere, and after between 2 and 10 hours at temperature, and separating the solid titanium metal with a diminished oxygen content from the molten reaction mixture.

30

#### References Cited in the file of this patent

##### UNITED STATES PATENTS

|              |                   |                |
|--------------|-------------------|----------------|
| 2,707,679    | Lillendahl et al. | May 3, 1955    |
| 35 2,718,464 | Gross et al.      | Sept. 20, 1955 |
| 2,723,182    | Sibert et al.     | Nov. 8, 1955   |
| 2,793,097    | McKenna           | May 21, 1957   |

##### FOREIGN PATENTS

|            |               |               |
|------------|---------------|---------------|
| 40 723,880 | Great Britain | Feb. 16, 1955 |
|------------|---------------|---------------|